

June 6, 1967

W. C. SIEVERT

3,323,940

METHOD FOR PRODUCING SMOOTH GALVANIZED SHEET

Filed Jan. 20, 1964



Inventor  
William C. Sievert  
Fay Merrion, Smith & Marshall  
Attorneys

**1**

3,323,940  
**METHOD FOR PRODUCING SMOOTH  
GALVANIZED SHEET**

William C. Sievert, Chesterton, Ind., assignor to Inland Steel Company, Chicago, Ill., a corporation of Delaware

Filed Jan. 20, 1964, Ser. No. 338,860  
3 Claims. (Cl. 117—114)

The present invention relates generally to processes for galvanizing flat, ferrous base material, and more particularly to a process for producing galvanized, flat, ferrous base material having a smooth, non-spangled, light gray, readily paintable surface coating primarily of zinc and having an iron content which is uniform along the entire area of the coated surface.

The production of smooth, readily paintable, non-spangled, galvanized strip having a surface coating of zinc alloyed with iron has been described generally in Mehler et al. U.S. Letters Patent No. 3,056,694. It is desirable that the iron content in the coating be uniform along the entire area of a coated surface on a strip and that this uniformity be consistent from strip to strip. The process of the present invention produces a coating of the type described generally in Mehler, and in addition produces a coating which is uniform from one end of a continuous strip to the other, and from one side edge of the strip to the other, as well as from continuous strip to continuous strip, no matter at what date the strip is made.

In addition to optimizing coating uniformity, the process of the present invention also imparts economies and minimizes the investment in equipment to an extent not available with processes lacking the features of the present invention.

Other features and advantages are inherent in the process claimed and disclosed or will become apparent to those skilled in the art from the following detailed description in conjunction with the accompanying diagrammatic drawing wherein:

FIGURE 1 is a schematic representation of apparatus suitable for carrying out an embodiment of a process in accordance with the present invention; and

FIGURE 2 is a plan view of flat, ferrous base galvanized material.

Basically, a strip to be treated in accordance with the present invention is initially coated, preferably in the manner described in detail in U.S. Letters Patent No. 2,110,898, by a process conventionally known as the Sendzimir type of process. After coating with zinc, the strip is subjected to a post heating or galvannealing step which promotes diffusion of iron from the ferrous base material into the zinc coating. As a result of this post heating step, the galvanized coating changes its appearance from a bright, spangled one to a non-spangled, smooth, light gray appearance. A product of this type, and with a uniform coating having an iron content between 4 and 7 wt. percent of the final coating, is the end result of a process practiced in accordance with the present invention, and now to be described in detail.

Initially, there is provided a coil of ferrous base flat material, such as steel strip, having a composition of the type conventionally used for galvanizing purposes (e.g., see the compositions listed on pages 666-7 in *The Making, Shaping and Treating of Steel*, 1957, United States Steel Corp., Pittsburgh, Pa.). The thickness of the base material may be any one of the conventional thicknesses

**2**

normally utilized for producing galvanized flat material (e.g., 10-24 gauge).

Referring to FIGURE 1, a steel strip 12 from a coil 11 is fed through an oxidizing furnace 13 in which the strip 12 is heated under oxidizing conditions to produce a thin, uniform oxide coating on the strip. The strip then passes through a furnace 14 containing a reducing atmosphere in which the oxide coating produced in furnace 13 is reduced to a tightly adhering layer of base metal free of oxides and other impurities. From reducing furnace 14 the strip passes over a roller 15 and into a hood or spout 16 leading from reducing furnace 14 to a point below the surface of a bath of molten zinc 17 contained in a pot 25. The molten zinc bath contains 0.05-0.30 wt. percent aluminum, with the preferable amount of aluminum being 0.13-0.18 wt. percent.

Spout 16, by extending below the surface of the molten zinc 17, forms an effective seal against the entry into reducing furnace 14 of oxidizing gases located above the surface of the molten zinc 17.

An important feature of the present invention is that the immersion temperature of strip 12, i.e., the temperature at which the strip enters the pot of molten zinc 17, is no greater than 900° F. An immersion temperature over 900° F. will over-promote diffusion of iron from the ferrous base into the zinc coating to such an extent that the final iron content in the zinc coating cannot be controlled to the degree necessary to produce the desirable light gray, non-spangled, smooth, adhering coating. A strip immersion temperature greater than 900° F. can cause overalloying to occur to such an extent that a dark gray, brittle coating will occur on the ferrous base strip, and the material will be unsuitable for bending or other deforming purposes.

There is no specified minimum immersion temperature for the strip, as there is a maximum temperature, although the strip will be at least above room temperature inasmuch as it has passed through two furnaces 13, 14 before entering zinc pot 25.

The purpose of the aluminum in the molten zinc is to retard or slow down diffusion of iron from the ferrous base into the zinc coating so that control can be exercised over the proportion of iron in the coating. As used herein, the term "traces of aluminum" means an amount of aluminum sufficient to enable satisfactory control to be exercised within the other conditions prevailing during the process. As indicated above, it has been conventional to utilize 0.05-0.30 wt. percent aluminum in the molten zinc, with a preferable aluminum content being 0.13-0.18 wt. percent. Both of these ranges are contemplated within the term "traces of aluminum."

Following immersion of strip 12 in zinc pot 25, the strip passes around a sinker roll 19, and then out of zinc bath 17 and through coating rolls 20 partially immersed in bath 17 and which are used to control the thickness of the zinc coating on the strip. Conventionally, the weight of the zinc coating on a single given surface of galvanized, flat ferrous base material is 0.1-1.0 ounce per square foot. In a typical galvanizing operation, a coating on one surface might be about 0.4-0.5 ounce per square foot for the one surface. Oftentimes, the coating weight on one surface differs from the coating weight on the other surface, depending upon the purpose for which the strip is to be utilized. In contrast, in a process in accordance with the present invention the coating weights must be con-

trolled so that they are the same on both surfaces of the strip.

In the process of the present invention, not only is the weight of the zinc coating controlled generally, but also, an important feature is the control of variations in coating weight from the front edge 26 to the rear edge 27 of strip 12, as well as of variations in coating weight from one side edge 28 to another side edge 29 (FIG. 2). In accordance with the present invention, the variation should not exceed  $\pm 0.05$  ounce per square foot on a given surface. Otherwise there will be either underalloying or overalloying, as well as the correct amount of alloying, at various localized areas on any given surface of any given strip. Such variations are undesirable because they result in fabricating difficulties or early failures of a localized portion of an object made out of the strip. Because of the step of controlling the variation in coating weight within  $\pm .05$  ounce per square foot, there are no such localized areas of underalloying or overalloying on a surface of flat galvanized material produced in accordance with the present invention.

Variations in coating weight along a given surface may be controlled by employing a number of techniques familiar to those skilled in the art and including: adjusting the tension of the coating rolls 20 on the strip; adjusting the depth of the coating rolls in the zinc bath; changing the number and depth of grooves with which the coating rolls are conventionally provided; maintaining the grooves free of accumulations of zinc dross; and adjusting the temperature of the zinc bath.

After coating, the next step in the process is to move the strip through alloying furnace 21 which may be fired in any conventional manner. An important feature of the present invention is that the furnace provide a temperature and have a heating capacity such that the strip is heated, at a strip heating rate of 25-30° F. per second, to a maximum strip temperature between 1000° and 1100° F., to promote diffusion of iron from the ferrous base strip into the coating. With this combination of heating rate and maximum strip temperature, the heating operation can be performed without holding the strip for any length of time at the maximum strip temperature; and upon attaining said maximum strip temperature, the strip may be immediately subjected to a cooling operation. This is economically advantageous because it enables utilization of a relatively small furnace length and a relatively rapid strip speed.

Heating to a maximum strip temperature below 1000°-1100° F. will produce undesirable underalloying whereas heating above that range will produce undesirable overalloying, when the other conditions of the process of the present invention are being practiced; and it is important to practice all of these conditions in order to obtain the desired economies of operation and equipment investment.

Immediately upon attainment of the maximum strip temperature (1000-1100° F.), the strip is cooled, without holding at the maximum strip temperature, to a strip temperature of 800° F. The cooling rate is controlled, between the maximum strip temperature and 800° F., to diffuse iron from the flat ferrous base strip into the coating until the amount of iron in the coating is between 4 and 7 wt. percent of the final coating. Although, in accordance with the present invention, the strip immersion temperature, the heating rate and the maximum strip temperature may be essentially the same from strip to strip, the desired thickness of the coating will vary, so that the actual cooling rate will vary with the thickness of the zinc coating. For example, assuming a coating thickness of 0.4-0.5 ounce of zinc per square foot on one surface, the cooling rate between the maximum strip temperature and 800° F. should be between 12 and 14° F. per second. With a thicker coating the cooling rate would be slower, and with a thinner coating the cooling rate would be faster. However, by assuring that the immersion temperature of the ferrous strip is below 900° F., and by as-

suring a heating rate of 25-30° F. per second and a maximum strip temperature of 1000-1100° F., the desired amount of iron in the zinc coating (between 4 and 7 wt. percent) can be obtained for virtually any thickness of coating within the thickness range conventionally utilized on galvanized flat base material (0.1-1.0 ounce per square foot on a given surface), merely by cooling to 800° F. using a cooling rate which is commercially practicable.

After the strip has been cooled from the maximum strip temperature to 800° F., utilizing a cooling rate to produce an iron content in the coating between 4 and 7 wt. percent, the strip is cooled rapidly from 800° F. at a rate sufficiently rapid to prevent further diffusion of iron into the coating. Once the temperature of the strip is cooled substantially below 800° F., little further diffusion of iron will occur. Therefore, it is important that the temperature be rapidly reduced below 800° F. immediately upon attainment of the desired amount of iron in the coating. This rapid cooling may be performed utilizing a stream of air or water directed against the coating or by any other method which will reduce the temperature of the strip rapidly enough to prevent further diffusion of iron.

The cooling operations may be performed in one or more cooling chambers 22 in which the strip is cooled by means such as a stream of cold air or a fine spray of water. The strip then passes over a roller 23 and subsequently typically proceeds to a coiling operation.

By utilizing a cooling operation of the type described, wherein the strip cooling rate is controlled down to 800° F. so as to promote diffusion of iron, and then the strip is cooled rapidly once it reaches 800° F. to prevent diffusion of iron; and by utilizing a strip immersion temperature, a strip heating rate and a maximum strip temperature within the respective ranges described above, the necessity of holding the strip at maximum strip temperature is eliminated. Because the strip need not be held for any length of time at the maximum strip temperature, it is not necessary to provide long, expensive furnaces.

Thus, in accordance with the present invention, there is produced a smooth, non-spangled, light gray galvanized coating on a flat ferrous base strip; and this coating is readily paintable, and has a uniform iron content from front edge to rear edge of any given strip, as well as from side edge to side edge of any given strip. In addition, the coating is produced utilizing a process which is economical, efficient and readily controllable.

The foregoing detailed description has been given for clearness of understanding only, and no unnecessary limitations should be understood therefrom, as modifications will be obvious to those skilled in the art.

What is claimed is:

1. A process for producing flat, galvanized ferrous strip having a uniform, smooth, non-spangled, light gray surface coating, said process comprising the steps of:
  - 55 immersing a flat ferrous base strip, with each surface free of oxides and other impurities and having a strip temperature below 900° F., into a bath of molten zinc containing traces of aluminum;
  - coating each surface of said base strip with the same thickness of said zinc, between 0.1 and 1.0 ounce per square foot of said zinc;
  - controlling the variation in said zinc coating on a surface, from side to side and from front edge to rear edge of the strip, to  $\pm .05$  ounce per square foot;
  - heating the coated strip, at a strip heating rate of 25-30° F. per second, to a maximum strip temperature between 1000°-1100° F. to promote the diffusion of iron from said ferrous base strip into said coating;
  - cooling said strip immediately upon attainment of said maximum strip temperature, without holding at said maximum strip temperature, to a strip temperature of 800° F.;
  - controlling the cooling rate, between said maximum strip temperature and 800° F., to diffuse iron from

said flat ferrous base strip into the coating in an amount of iron between 4 and 7% of the final coating weight;  
and then cooling said strip upon attainment of said 5 800° F. to a temperature below 800° F. at a cooling rate sufficient to prevent further diffusion of iron into said coating.

2. A process as recited in claim 1 wherein:  
said strip is coated on each surface thereof with .4-.5 ounce of zinc per square foot;  
and said coated strip is cooled from said maximum 10 temperature to 800° F., at a cooling rate of 12°-14° F. per second.

3. A process as recited in claim 1 wherein said cooling rate from 800° F. to a temperature below 800° F. is faster than said cooling rate from said maximum strip temperature to 800° F.

#### References Cited

#### UNITED STATES PATENTS

|           |         |               |       |           |
|-----------|---------|---------------|-------|-----------|
| 3,056,694 | 10/1962 | Mehler et al. | ----- | 117—114   |
| 3,058,840 | 10/1962 | Kerr et al.   | ----- | 117—114 X |
| 3,177,088 | 4/1965  | Sievert       | ----- | 117—114   |

ALFRED L. LEAVITT, *Primary Examiner.*

R. S. KENDALL, *Assistant Examiner.*